

# UNITED STATES PATENT OFFICE.

DAVID J. HAUSS, OF AURORA, INDIANA; BARBARA HAUSS, ADMINISTRATRIX OF SAID  
DAVID J. HAUSS, DECEASED, ASSIGNOR TO F. W. GALBRAITH.

## ALLOY.

1,293,426.

Specification of Letters Patent.

Patented Feb. 4, 1919.

No Drawing.

Application filed June 26, 1916. Serial No. 105,866.

To all whom it may concern:

Be it known that I, DAVID J. HAUSS, a citizen of the United States, residing at Aurora, in the county of Dearborn and 5 State of Indiana, have invented certain new and useful Improvements in Alloy, of which the following is a specification.

My invention relates to improvements in metallic alloy. One of its objects is to provide an alloy having great strength combined with a low fusing point. Another object is to provide an alloy having a high degree of fluidity when fused, combined with strength when solid. Another object 10 is to provide an alloy of great strength and capable of resisting corrosion from exposure to the atmosphere, moisture or other corrosive agencies. Another object is to provide an alloy of great strength and of 15 comparatively low specific gravity.

My invention also comprises certain details of proportion and procedure, all of which will be set forth in the following specification.

25 One method of producing my new alloy is as follows:

Metallic aluminum and metallic zinc in substantially the proportions of 72 parts aluminum and 24 to 25 parts of zinc are 30 melted together in a crucible, using a protecting film or covering of granulated carbon, preferably charcoal. When the aluminum and zinc have fused together, which should occur at from 1100 to 1200 degrees 35 F, I quickly and carefully add a previously prepared capsule containing 3 parts metallic copper and  $\frac{1}{4}$  to  $\frac{1}{2}$  part of metallic magnesium. The effect of adding the contents of 40 the capsule is to greatly increase the fluidity and to reduce the fusing point. The metallic copper remains as a component of the alloy, but the magnesium is believed not to enter to any extent as a component of the alloy, but instead to serve the purpose of 45 removing any metallic oxids from the body of the alloy. It is therefore probable that metallic calcium or similar metal having a stronger affinity than aluminum for oxygen, could be substituted in substantially like 50 proportion for the magnesium mentioned.

My improved alloy can also be produced electrolytically by employing one or a plurality of anodes of carbon and metal and preferably a single cathode so that one of 55 the metals, say the aluminum or zinc may

be derived by electrolysis from the electrolyte while the others are transferred from the anode or anodes in quantity to produce an alloy of the desired proportions by regulating the amount of current through said 60 respective anodes. When produced electrolytically the magnesium or its equivalent is dispensed with as the current serves to reduce or prevent the formation of any metallic oxids in the alloy at the cathode. 65

My new alloy possesses the following characteristics, the metals are present in substantially the following proportions:

|                      |    |
|----------------------|----|
| 72 parts aluminum,   | 70 |
| 24 to 25 parts zinc, |    |
| 3 parts copper.      |    |

It melts at approximately 1000° F., and is very fluid, as distinguished from "pasty" so as to adapt it to the formation of thin, 75 sharp and strong castings. Its tensile strength is in excess of 40,000 pounds per square inch. Its specific gravity is not materially greater than that of metallic aluminum. 80

The proportion of copper may be varied slightly; an increase in the amount of copper increases the tensile strength, but also raises the melting point, while a decrease of the amount of copper decreases the strength but 85 does not correspondingly lower the melting point.

An increase in the proportion of zinc decreases the tensile strength and does not in other respects improve the qualities of the 90 alloy. A decrease in the quantity of zinc does not improve the qualities of the alloy either by increasing the strength or reducing the melting point.

It is believed that the low melting point 95 and great strength of my new alloy is due to the formation of a definite chemical compound when combined in substantially the proportions specified as distinguished from a simple alloy or metallic solution such as 100 commonly designated by the term alloy.

The capsule employed to introduce the copper and magnesium may be of gelatin, cardboard, or other material which will not affect the composition of the alloy, and is 105 employed chiefly to assist in introducing the metals, which are more or less finely divided to a point below the surface of the fused metal before reaction of a chemical nature commences.

Having described my invention or discovery, what I claim is:

An alloy composed of substantially seventy-two parts aluminum, twenty-four to twenty-five parts zinc, and three parts copper, said alloy being practically free from the oxids of said metals.

In testimony whereof I have affixed my signature in the presence of two witnesses.

DAVID J. HAUSS.

Witnesses:

C. W. MILES,  
W. THORNTON BOGERT.